

## UNITED STATES PATENT OFFICE

2,663,613

## PROCESS FOR COLORING NYLON FIBER

Joseph Whitton Gibson, Jr., Penns Grove, N. J., assignor to E. I. du Pont de Nemours and Company, Wilmington, Del., a corporation of Delaware

No Drawing. Application May 10, 1950,  
Serial No. 161,267

8 Claims. (Cl. 8—37)

1

In copending application Serial No. 161,265 of even date herewith, I am describing and claiming a general method for improving the process of coloring heat-stable, hydrophobic textile fiber such as nylon, polyacrylonitrile fiber and polyethylene terephthalate fiber. The improvement consists in subjecting the fiber, after impregnation with the selected coloring material and drying, to a heat treatment in the absence of moisture at a temperature between 180° and 250° C. This invention is in the nature of a species under the above general case, and concerns itself primarily with nylon fiber.

Nylon can be dyed with many classes of dyes; however, relatively long dyeing times are required and the dyeings are usually not level. Level dyeings are obtained on nylon filament only with dispersed colors which are suitable for the dyeing of cellulose acetate, but here the dyeings have insufficient light- and wash-fastness for many practical uses.

Accordingly, it is an object of this invention to provide a process for coloring nylon fiber under novel conditions whereby to produce uniform dyeings and to accelerate fixation to a point where the process becomes adapted for continuous operation. Additional important objects of this invention will appear as the description proceeds.

These objects are achieved according to this invention by subjecting the nylon fiber to a special heat-treatment after impregnating the same, in ordinary manner, with the selected coloring material from an aqueous medium. For instance, the fiber may be padded with an aqueous solution or suspension of the selected coloring material (that is, dye or intermediate for dye), or it may be printed with a thickened, aqueous printing paste containing said coloring material. The impregnated fiber is then dried, and then subjected to a heat treatment at a temperature of between 180° and 230° C., for a brief interval of time. This time interval is usually less than 1 minute, and may in some cases be as brief as 5 seconds. I find, however, that nylon fiber withstands the prescribed range of temperature for considerably longer periods. It is therefore possible to practice my invention with longer heating periods, say up to 2 or even 3 minutes, provided the system of apparatus available is such as to make continuous operation under these conditions economical.

The application of my invention to nylon results first of all in a speedier fixation of the color upon the fiber, thereby adapting the process

2

better for continuous operation, that is the dyeing of fabric from a continuous roll. Also, with some classes of dyestuffs, especially acid wool dyestuffs, where the ordinary processes produce streaky, uneven dyeings upon nylon, my invention produces uniform dyeings, pleasing in appearance.

In general, the colors which are applicable by my invention are those which will dye nylon from an aqueous dye bath at the boil either neutral or slightly acid (pH 7 to pH 3). These include the following classes of colors:

10 Acid wool dyes. (These are usually azo dyes possessing SO<sub>3</sub>H groups and simple anthraquinone compounds having sulfonic acid groups.)

15 Metallized, water-soluble and water-insoluble azo dyes. (These are usually ortho-hydroxy-azo dyes, aftertreated with compounds of chromium, nickel, copper or other polyvalent metal.)

20 Cellulose-acetate dyes. (These are generally azo dyes free of SO<sub>3</sub>H groups, and simple anthraquinone derivatives having amino or hydroxy groups, but no SO<sub>3</sub>H groups.)

25 Basic dyes (whether water-soluble or not).

28 Direct cotton dyes (usually azo dyes having SO<sub>3</sub>H or SO<sub>3</sub>Na groups).

Sulfur dyes in conjunction with sodium sulfide. (The latter aids in dissolving the sulfur color, forming the so-called sulfide vat.)

30 Mercaptolated or thiocyanated dyes, that is dyes which while belonging on their own merits to some other standard class are converted into sulfide-vattable dyes by the introduction of SH groups or SCN groups. See for instance, Fox U. S. P. 2,369,666 and Haddock U. S. P. 2,342,662.

35 Furthermore, I find that in lieu of the finished dyestuff or pigment I often may employ intermediates adapted to yield the desired coloring compound upon heating. For instance, I may impregnate the fiber with a soluble, leuco ester of a vat dye. Then in the heating step the leuco ester becomes converted to the oxidized or keto form. Or again, I may pad the fiber with the components of an azo dye, for instance an azoic coupling component and an aryl amine and subject the impregnated fiber, after drying, to a heat treatment as above described, to effect penetration of the components into the fiber. When the fiber is then treated with an aqueous diazotizing bath, with or without subsequent alkalization (Cf. British Patent No. 629,452), an azo dye is formed within the fiber.

40 The exposure to heat may be achieved in any available apparatus suitable for supplying dry heat at the temperature interval of 180° to 230°.

## 3

C. For operating on a continuous fabric or yarn, a heated drum will naturally be the most convenient form. Other methods, however, may be resorted to, for instance passing the fabric through a molten metallic bath (such as Cerro-bend, a low-melting lead alloy), through a flue drier, or under infra-red radiation.

Following the heat treatment, the fabric is preferably subjected to a soaping operation to remove any residual, loosely adhering, superficial pigment particles. The fiber is then rinsed and dried.

Without limiting my invention, the following examples are given to illustrate the details of operation. Parts mentioned are by weight.

## Example 1

A 2% solution of an acid green anthraquinone dye, C. I. 1078, was padded onto filament nylon fabric. The fabric was dried and passed through a flue drier, maintained at 215° C., at such a rate that the exposure time was 30 seconds. The so-obtained dyeing was soaped for five minutes at 71° C. in a solution containing 5 g./l. of sodium oleate. A level, medium green shade was obtained which exhibited good washing-, light- and crocking-fastness. A similar dyeing prepared by dyeing in a similar color solution at the boil exhibited similar fastness properties but contained pronounced warp streaks.

Other water-soluble colors applied to nylon by the same procedure were:

| Color Employed                                                           | Shade Obtained |
|--------------------------------------------------------------------------|----------------|
| Acid Violet, C. I. 1080                                                  | Violet.        |
| Acid Blue, C. I. 1088                                                    | Blue.          |
| Acid Blue, C. I. 289                                                     | Dark Blue.     |
| The p-tolyl derivative of the dyestuff of Example II, U. S. P. 2,124,688 | Brown.         |

## Example 2

A 5% aqueous solution of the dyestuff of Example 1, U. S. P. 1,724,663 was padded onto a nylon fabric. The fabric was dried and passed through a flue drier, maintained at 215° C., at such a rate that the exposure time was forty seconds. The dyeing was soaped as described above. A level, medium orange shade was obtained which exhibited good washing-, light- and crocking-fastness.

In a similar manner, except for using suspensions in lieu of solutions where the color was insoluble, the following colors were applied to nylon with the following results:

|                                                                                                  |         |
|--------------------------------------------------------------------------------------------------|---------|
| The half-chromed form of the dyestuff of Example 2, U. S. P. 1,623,005                           | Orange  |
| 4 - (o-hydroxy phenylazo) - 3-methyl-1-phenyl-5-pyrazolone, nickelized                           | Yellow  |
| $\alpha$ - (2 - nitro - p - tolylazo) - aceto-acetanilide                                        | Yellow  |
| Vat dye, C. I. 1228                                                                              | Red     |
| Dyestuff made according to Example 35, U. S. P. 2,212,928, using 1-amino-4-anilino-anthraquinone | Scarlet |

## Example 3

An aqueous bath was prepared containing 5% by weight of sodium dichromate and 5% of the diazo dye prepared by coupling 2-amino-4-nitrophenol and 1-amino-5-naphthalene sulfonic acid to m-phenylene diamine. Nylon fabric was padded with this solution, dried, and passed between two metal surfaces, maintained at 205° C., in such a way that the exposure time was 20 75 71° C. with 5 g./l. of sodium oleate. An olive

## 4

seconds. The fabric was soaped for 5 minutes at 71° C. with 5 g./l. of sodium oleate. A brown dyeing was obtained which exhibited excellent crock-fastness and fair light-fastness.

## Example 4

A 5% aqueous dispersion of 4-(4'-nitrophenylazo)-2,5-xylidine was prepared by warming the dyestuff paste and water at 60° C. with stirring until completely dispersed. The dispersion was then padded onto a nylon fabric. The squeeze rolls were adjusted to give a pick-up of 30%. The fabric was then dried and passed through a flue drier, maintained at 190° C., in such a way that the exposure time was 30 seconds. It was then soaped as described above. A bright orange dyeing was obtained which exhibited good crocking- and fair washing- and light-fastness.

Other colors applied to nylon by the same procedure and with substantially equal results were:

| Color Employed                  | Shade Obtained |
|---------------------------------|----------------|
| 1-amino-4-hydroxy-anthraquinone | Red.           |
| 1,4,5,8-tetramino-anthraquinone | Blue.          |

## Example 5

30 A paste containing the following ingredients was prepared:

|                        | Parts |
|------------------------|-------|
| Acid green, C. I. 1078 | 4     |
| Water                  | 26    |
| Thiodiglycol           | 10    |
| Hydroxyacetic acid     | 10    |
| Textile gum            | 50    |
| Total                  | 100   |

40 Nylon fabric was printed with this paste and dried. It was then passed continuously between two metal surfaces maintained at 225° C. in such a way that the exposure time was forty seconds. The fabric was soaped for 5 minutes at 71° C. with 5 g./l. of sodium oleate. A green print was obtained that was bluer but duller than a similar print by standard printing methods.

Other colors printed successfully on nylon by the same procedure were:

| Color Employed                                                               | Shade Obtained |
|------------------------------------------------------------------------------|----------------|
| 1-amino-4-(2-sulfo-p-toluidino)-2-anthraquinone-sulfonic acid, disodium salt | Blue.          |
| The dyestuff of Example 1, U. S. P. 1,724,663                                | Orange.        |
| The half-chromed form of the dyestuff of Example 2, U. S. P. 1,623,005       | Do.            |

## Example 6

60 A mixed dye bath was prepared as follows:

|                                                                                         | Parts |
|-----------------------------------------------------------------------------------------|-------|
| Half-chromed azo dye of Example 2, U. S. P. 1,623,005                                   | 2.25  |
| Direct Yellow (C. I. 364)                                                               | 0.75  |
| 1 - amino - 4 - (m - methylol - anilino) - 2 - anthraquinone sulfonic acid, sodium salt | 2.25  |
| Water                                                                                   | 100   |

70 The mixture was warmed to 60° C. and stirred until the dyes were completely dissolved. Nylon tow was then padded in this solution, dried and passed through a dryer maintained at 225° C. in such a way that the exposure time was 60 seconds. The tow was soaped for 5 minutes at 71° C. with 5 g./l. of sodium oleate. An olive

dyeing was obtained which exhibited good crocking-, light- and wash-fastness.

A similar dyeing is obtained if using raw stock instead of tow by the above procedure.

*Example 7*

A 1% solution of anilide of beta-oxy-naphthoic acid in "Cellosolve" (ethylene glycol monoethyl ether) was padded onto nylon fiber and dried. A 5% solution of m-nitro aniline in 95% ethanol was over-padded on the above padding and dried. The fabric was then passed between two metal surfaces maintained at 205° C. in such a way that the exposure time was 30 seconds. It was then treated for five minutes at 100° C. with a solution of 3 g./l. sodium nitrite and 3.7 g./l. hydrochloride acid. A medium orange shade was obtained which exhibited excellent crock-fastness.

The same fibers were also dyed by the same procedure except for selecting different amines, with the following results:

| Amine Selected      | Shade Obtained |
|---------------------|----------------|
| 2-nitro-p-toluidine |                |
| 4,4'-di-o-anisidine | Red. Violet.   |

It will be clear from the above examples that my invention is applicable with a wide variety of water-soluble and water-insoluble dyestuff or, indeed, with organic substances which are not dyestuffs per se but are convertible into dyestuffs when heated by themselves or in the presence of oxidizing agents.

The advantages, as already noted, are in general accelerated fixation time, and uniform, even dyeings in cases where these have been wanting. Furthermore, dyeing in my invention is generally achieved without resort to swelling agents, resins or other special assistants.

Finally, it is well known that nylon generally requires a heat-setting treatment to set the fiber. In ordinary practice, this operation requires special handling in a special setting of apparatus. By the process of my invention, however, this extra operation may be dispensed with, since it is possible to achieve both dyeing and heat-setting in one continuous operation.

The class of nylon fibers with which this invention deals is well known in the art, and refers to a group of film-forming polymeric amides. See for instance, Carothers, U. S. P. 2,071,250, 2,071,253 and 2,130,948.

I claim as my invention:

1. A process for continuously coloring nylon fiber, which comprises impregnating the same continuously with an organic coloring matter from an aqueous medium, drying continuously the impregnated fiber, and then continuously

subjecting the same to a heat treatment in the absence of moisture at a temperature not less than 190° C. and not greater than 230° C., for a period of time of from 20 to 60 seconds, whereby to effect fixation of the color within the fiber.

2. A process for coloring a continuous length of nylon fabric which comprises impregnating continuously fresh portions of said fabric with an aqueous suspension of an organic coloring matter, drying the impregnated portions and then subjecting them to a heat treatment in the absence of moisture at a temperature not less than 190° C. and not greater than 230° C., for a period of time of from 20 to 60 seconds, whereby to effect fixation of the color within the fiber.

3. A process as in claim 2, the impregnation consisting of padding the nylon fiber in an aqueous bath containing said organic coloring material, and the heating step being followed by washing to remove superficially disposed surplus coloring material.

4. A process as in claim 3, the aqueous bath comprising a dispersion of a water-insoluble cellulose-acetate dye.

5. A process as in claim 3, the aqueous bath comprising a metallized azo dye.

6. A process as in claim 3, the aqueous bath comprising a solution of an acid dye.

7. A process as in claim 3, the aqueous bath comprising an aqueous solution of a water-soluble basic dye.

8. A process as in claim 3, the aqueous bath comprising an aqueous sulfide-vat of a sulfur color.

JOSEPH WHITTON GIBSON, JR.

References Cited in the file of this patent

UNITED STATES PATENTS

| Number    | Name    | Date          |
|-----------|---------|---------------|
| 2,080,254 | Dreyfus | May 11, 1937  |
| 2,474,890 | Croft   | July 5, 1949  |
| 2,532,437 | Baker   | Dec. 5, 1950  |
| 2,543,316 | Feild   | Feb. 27, 1951 |
| 2,577,846 | Feild   | Dec. 11, 1951 |

FOREIGN PATENTS

| Number  | Country | Date          |
|---------|---------|---------------|
| 378,566 | Italy   | Feb. 15, 1940 |
| 913,158 | France  | May 20, 1946  |

OTHER REFERENCES

Silk Journal and Rayon World for February 1947, page 55.

"Technical Bulletin" for June 1949, volume 5, Number 2, pages 82 to 103, published by Du Pont, Wilmington, Delaware.

Rayon Textile Monthly for September 1946, page 140 (496).

Textile Colorist for December 1943, pages 551 to 553.

**Dedication**

2,663,613.—*Joseph Whitton Gibson, Jr., Penns Grove, N.J. PROCESS FOR COLORING NYLON FIBER. Patent dated Dec. 22, 1953. Dedication filed July 29, 1963, by the assignee, E. I. du Pont de Nemours and Company.*  
Hereby dedicates to the people of the United States the entire term of said patent.

[*Official Gazette October 22, 1963.*]